

## UNITED STATES PATENT OFFICE

1,930,341

## ZINC BASE DIE CASTING ALLOY

John R. Freeman, Jr., Waterbury, Conn., assignor to The American Brass Company, Waterbury, Conn., a corporation of Connecticut

No Drawing. Application August 29, 1931  
Serial No. 560,227

2 Claims. (Cl. 75—1)

This invention relates to zinc base die casting alloys and has for its object a new and improved alloy for die castings.

Heretofore the design of die casting machines has been such that the mechanism is to a great extent completely immersed in the molten alloy to be cast. The casting mechanism is of necessity made of steel and cast iron both of which are attacked by molten zinc and zinc base alloys with the exception of zinc alloys containing more than 0.25% aluminum, the presence of which greatly reduces the attack of the steel and iron parts by the zinc. Aluminum has thus heretofore been an essential requirement in die casting alloys.

There have recently become available die casting machines in which the melting chamber is separated from the casting mechanism. As a result it is possible to economically die cast products of zinc base alloy which do not contain aluminum.

In the preparation of such products zinc of commercial quality has been used such as zinc of quality defined as No. 1 or high grade by the American Society for Testing Materials in their specification No. B6-18. High grade zinc of this quality may contain as much as 0.07% lead and cadmium respectively and 0.03% of iron.

Zinc base alloys containing from about 0.5 to about 15% of copper prepared from high grade zinc as above specified are open to the objection that the alloys develop what is commonly termed "hot shortness" in the die casting process more particularly in the manufacture of the more intricate castings.

I have discovered that this "hot shortness" when present in alloys of zinc and copper is due to the presence of impurities, more particularly lead and cadmium, usually found in high grade

zinc as above specified. I have discovered however, that by reducing the impurity content of zinc base copper alloys, in particular the lead and cadmium content, castings of the above alloys may be produced which are free from the objection of hot shortness and therefore are suitable for a wide range of applications where the alloys previously discussed prepared from high grade zinc containing normal impurities are not suitable.

Based on this discovery my invention resides in the provision of a new zinc base die casting alloy containing approximately 0.50 to 15% of copper and balance zinc metal of special purity such that the resultant alloy is free from elements that cause hot shortness, in particular the elements lead and cadmium. More particularly the invention involves the provision of a new zinc base die casting alloy containing from about 0.5% to 15% of copper in which the zinc base is 75 of zinc metal containing total impurities not to exceed 0.02%. The above range of about 0.50% to 15% copper produces a series of useful alloys, but the preferred range is from about 2% to about 6% copper and the balance zinc.

Having thus set forth the nature of my invention, what I claim is:

1. As a new article of manufacture a metallic product comprising a die casting made of a zinc base alloy containing from about 0.5 percent to 85 about 15 percent copper and the remainder zinc metal containing 99.98 percent or more zinc.

2. As a new article of manufacture a metallic product comprising a die casting made of a zinc base alloy containing from about 2 percent to 90 about 6 percent copper and the remainder zinc metal containing at least 99.98 percent zinc.

JOHN R. FREEMAN, JR.

40

95

45

100

50

105

55

110